



US008841243B2

(12) **United States Patent**  
**Tobias et al.**

(10) **Patent No.:** **US 8,841,243 B2**  
(45) **Date of Patent:** **\*Sep. 23, 2014**

(54) **NATURAL GAS ENGINE LUBRICATING OIL COMPOSITIONS**

(75) Inventors: **Melanie F. Tobias**, Pleasant Hill, CA (US); **Jon F. Von Staden**, San Antonio, TX (US)

(73) Assignee: **Chevron Oronite Company LLC**, San Ramon, CA (US)

(\*) Notice: Subject to any disclaimer, the term of this patent is extended or adjusted under 35 U.S.C. 154(b) by 0 days.

This patent is subject to a terminal disclaimer.

(21) Appl. No.: **12/798,255**

(22) Filed: **Mar. 31, 2010**

(65) **Prior Publication Data**

US 2011/0245121 A1 Oct. 6, 2011

(51) **Int. Cl.**

**C10M 169/04** (2006.01)  
**C07C 309/62** (2006.01)  
**C10M 129/76** (2006.01)  
**C09K 15/08** (2006.01)  
**C10M 137/10** (2006.01)  
**C10M 141/10** (2006.01)  
**C10M 163/00** (2006.01)

(52) **U.S. Cl.**

CPC ..... **C10M 169/04** (2013.01); **C10M 163/00** (2013.01); **C10M 2203/1025** (2013.01); **C10M 2223/045** (2013.01); **C10N 2240/10** (2013.01); **C10M 2223/049** (2013.01); **C10M 2215/28** (2013.01); **C10M 2207/262** (2013.01); **C10N 2230/42** (2013.01); **C10M 2207/14** (2013.01); **C10M 2223/04** (2013.01); **C10M 2207/026** (2013.01); **C10N 2230/45** (2013.01); **C10M 169/045** (2013.01); **C10N 2230/06** (2013.01); **C10M 2219/022** (2013.01); **C10N 2220/021** (2013.01)

USPC ..... **508/291**; 508/390; 508/502; 508/584; 508/370; 508/421

(58) **Field of Classification Search**

USPC ..... 508/287, 110, 390, 502, 584, 370, 291, 508/421

See application file for complete search history.

(56) **References Cited**

U.S. PATENT DOCUMENTS

2,263,312 A 11/1901 Reed  
2,202,781 A 5/1939 Kennedy

(Continued)

FOREIGN PATENT DOCUMENTS

CN 1523088 A 8/2004  
CN 101671596 A 3/2010

(Continued)

OTHER PUBLICATIONS

The International Search Report dated Sep. 30, 2013 issued in counterpart Chinese Patent Application No. 201130011449.2.

(Continued)

*Primary Examiner* — Vishal Vasisth

(57) **ABSTRACT**

A natural gas engine lubricating oil composition is disclosed which comprises (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents.

**7 Claims, 1 Drawing Sheet**



| (56)                                                                                                                                            | References Cited |                 |                   |         |                   |
|-------------------------------------------------------------------------------------------------------------------------------------------------|------------------|-----------------|-------------------|---------|-------------------|
| U.S. PATENT DOCUMENTS                                                                                                                           |                  |                 |                   |         |                   |
| 2,174,110 A                                                                                                                                     | 9/1939           | Reed            | 3,567,637 A       | 3/1971  | Nishijima et al.  |
| 2,174,506 A                                                                                                                                     | 9/1939           | Fox             | 3,586,629 A       | 6/1971  | Otto et al.       |
| 2,174,508 A                                                                                                                                     | 9/1939           | Fox             | 3,591,598 A       | 7/1971  | Traise et al.     |
| 2,193,824 A                                                                                                                                     | 3/1940           | Lockwood et al. | 3,595,790 A       | 7/1971  | Norman            |
| 2,197,800 A                                                                                                                                     | 4/1940           | Henke et al.    | 3,595,791 A       | 7/1971  | Cohen             |
| 2,197,832 A                                                                                                                                     | 4/1940           | Reiff           | 3,629,109 A       | 12/1971 | Gergel et al.     |
| 2,197,835 A                                                                                                                                     | 4/1940           | Reiff           | 3,632,610 A       | 1/1972  | Schmitz           |
| 2,212,786 A                                                                                                                                     | 8/1940           | McQueen         | 3,646,730 A       | 3/1972  | Reid              |
| 2,213,360 A                                                                                                                                     | 9/1940           | Calcott et al.  | 3,666,730 A       | 5/1972  | Coleman           |
| 2,223,676 A                                                                                                                                     | 12/1940          | Dinsmure et al. | 3,666,732 A       | 5/1972  | Skoulchi et al.   |
| 2,228,598 A                                                                                                                                     | 1/1941           | Fox et al.      | 3,775,321 A       | 11/1973 | Tumquest et al.   |
| 2,239,974 A                                                                                                                                     | 4/1941           | Reed et al.     | 3,798,012 A       | 3/1974  | Le Suer           |
| 2,252,662 A                                                                                                                                     | 8/1941           | Reiff           | 3,798,163 A       | 3/1974  | Palmer            |
| 2,252,664 A                                                                                                                                     | 8/1941           | Reiff           | 3,850,822 A       | 11/1974 | Steere et al.     |
| 2,276,090 A                                                                                                                                     | 3/1942           | Reed            | 3,980,569 A       | 9/1976  | Pindar et al.     |
| 2,276,097 A                                                                                                                                     | 3/1942           | Salzberg        | 4,234,435 A       | 11/1980 | Meinhardt et al.  |
| 2,315,514 A                                                                                                                                     | 4/1943           | Fox             | 4,612,132 A       | 9/1986  | Wollenberg et al. |
| 2,319,121 A                                                                                                                                     | 5/1943           | Fox             | 4,746,446 A       | 5/1988  | Wollenberg et al. |
| 2,321,022 A                                                                                                                                     | 6/1943           | Fox             | 4,849,118 A       | 7/1989  | Stauffer et al.   |
| 2,333,568 A                                                                                                                                     | 11/1943          | Henke et al.    | 5,595,964 A       | 1/1997  | Bardasz           |
| 2,333,788 A                                                                                                                                     | 11/1943          | Holbrook et al. | 5,716,912 A       | 2/1998  | Harrison et al.   |
| 2,335,259 A                                                                                                                                     | 11/1943          | Calcott         | 5,726,133 A       | 3/1998  | Blahey et al.     |
| 2,337,552 A                                                                                                                                     | 12/1943          | Henke           | 6,001,780 A       | 12/1999 | Ho et al.         |
| 2,347,568 A                                                                                                                                     | 4/1944           | Kunert          | 6,147,035 A       | 11/2000 | Sougawa et al.    |
| 2,366,027 A                                                                                                                                     | 12/1944          | Henke           | 6,153,565 A       | 11/2000 | Skinner et al.    |
| 2,374,193 A                                                                                                                                     | 4/1945           | Grubb           | 6,165,235 A       | 12/2000 | Kolp et al.       |
| 2,383,319 A                                                                                                                                     | 8/1945           | Kharasch        | 6,174,842 B1      | 1/2001  | Gatto et al.      |
| 2,501,731 A                                                                                                                                     | 3/1950           | Mertes          | 6,281,179 B1      | 8/2001  | Skinner et al.    |
| 2,616,904 A                                                                                                                                     | 11/1952          | Asseff et al.   | 6,372,696 B1      | 4/2002  | Tipton            |
| 2,616,905 A                                                                                                                                     | 11/1952          | Asseff et al.   | 6,429,178 B1      | 8/2002  | Skinner et al.    |
| 2,616,906 A                                                                                                                                     | 11/1952          | Asseff et al.   | 6,449,179 B1      | 8/2002  | Skinner et al.    |
| 2,616,911 A                                                                                                                                     | 11/1952          | Asseff          | 6,440,905 B1      | 8/2002  | Epps et al.       |
| 2,616,924 A                                                                                                                                     | 11/1952          | Asseff et al.   | 6,596,672 B1      | 7/2003  | Carrick et al.    |
| 2,616,925 A                                                                                                                                     | 11/1952          | Asseff et al.   | 6,613,724 B2      | 9/2003  | Strickland et al. |
| 2,617,049 A                                                                                                                                     | 11/1952          | Asseff et al.   | 6,642,191 B2      | 11/2003 | Palazzotto et al. |
| 2,680,096 A                                                                                                                                     | 6/1954           | Walker et al.   | 6,727,208 B2      | 4/2004  | Wilk              |
| 2,714,092 A                                                                                                                                     | 7/1955           | Colnane et al.  | 6,756,348 B2      | 6/2004  | Palazzotto et al. |
| 2,777,874 A                                                                                                                                     | 1/1957           | Asseff et al.   | 7,309,681 B2      | 12/2007 | Cartwright        |
| 3,027,325 A                                                                                                                                     | 3/1962           | McMillen et al. | 2004/0142827 A1   | 7/2004  | Palazzotto et al. |
| 3,036,003 A                                                                                                                                     | 5/1962           | Verdol          | 2005/0054543 A1   | 3/2005  | Cartwright        |
| 3,036,971 A                                                                                                                                     | 5/1962           | Otto            | 2005/0070447 A1   | 3/2005  | Barnes et al.     |
| 3,172,892 A                                                                                                                                     | 3/1965           | Le Suer et al.  | 2005/0137098 A1   | 6/2005  | Le Cuent et al.   |
| 3,219,666 A                                                                                                                                     | 11/1965          | Norman et al.   | 2007/0027043 A1   | 2/2007  | Le Cuent          |
| 3,256,186 A                                                                                                                                     | 6/1966           | Greenwald       | 2007/0066495 A1*  | 3/2007  | Macpherson .....  |
| 3,271,130 A                                                                                                                                     | 9/1966           | Denig           | 2007/0111905 A1*  | 5/2007  | 508/192           |
| 3,272,746 A                                                                                                                                     | 9/1966           | Le Suer et al.  | 2007/0129263 A1   | 6/2007  | van Dam .....     |
| 3,275,554 A                                                                                                                                     | 9/1966           | Wagenaar        | 2007/0142239 A1   | 6/2007  | 508/273           |
| 3,282,835 A                                                                                                                                     | 11/1966          | Asseff          | 2008/0153722 A1*  | 6/2008  | Boffa et al.      |
| 3,312,618 A                                                                                                                                     | 4/1967           | Le Suer et al.  | 2008/0269089 A1   | 10/2008 | Boffa et al.      |
| 3,318,809 A                                                                                                                                     | 5/1967           | Bray            | EP 0351906        | 9/1992  | 508/149           |
| 3,320,162 A                                                                                                                                     | 5/1967           | Axe et al.      | EP 0927754        | 7/1999  |                   |
| 3,329,658 A                                                                                                                                     | 7/1967           | Fields          | EP 1104800 A2     | 6/2001  |                   |
| 3,342,733 A                                                                                                                                     | 9/1967           | Robbins et al.  | EP 1227145 A1     | 7/2002  |                   |
| 3,350,038 A                                                                                                                                     | 10/1967          | Oberlander      | EP 1439217 A1     | 7/2004  |                   |
| 3,368,396 A                                                                                                                                     | 2/1968           | Burkleo et al.  | GB 1368277        | 9/1974  |                   |
| 3,373,108 A                                                                                                                                     | 3/1968           | Woodle et al.   | JP 2927530        | 7/1999  |                   |
| 3,384,585 A                                                                                                                                     | 5/1968           | Gragson et al.  | JP 2004/107556    | 4/2004  |                   |
| 3,410,798 A                                                                                                                                     | 11/1968          | Cohen           | JP 2005/162968    | 6/2005  |                   |
| 3,438,757 A                                                                                                                                     | 4/1969           | Honnen et al.   | WO WO 2010/009036 | 1/2010  |                   |
| 3,449,250 A                                                                                                                                     | 6/1969           | Fields          |                   |         |                   |
| 3,454,555 A                                                                                                                                     | 7/1969           | Vander Voort    |                   |         |                   |
| 3,471,403 A                                                                                                                                     | 10/1969          | Le Suer et al.  |                   |         |                   |
| 3,488,284 A                                                                                                                                     | 1/1970           | Le Suer et al.  |                   |         |                   |
| 3,510,428 A                                                                                                                                     | 5/1970           | Didden et al.   |                   |         |                   |
| 3,523,082 A                                                                                                                                     | 8/1970           | Vienna et al.   |                   |         |                   |
| 3,565,804 A                                                                                                                                     | 2/1971           | Honnen et al.   |                   |         |                   |
| FOREIGN PATENT DOCUMENTS                                                                                                                        |                  |                 |                   |         |                   |
| EP 0351906                                                                                                                                      | 9/1992           |                 |                   |         |                   |
| EP 0927754                                                                                                                                      | 7/1999           |                 |                   |         |                   |
| EP 1104800 A2                                                                                                                                   | 6/2001           |                 |                   |         |                   |
| EP 1227145 A1                                                                                                                                   | 7/2002           |                 |                   |         |                   |
| EP 1439217 A1                                                                                                                                   | 7/2004           |                 |                   |         |                   |
| GB 1368277                                                                                                                                      | 9/1974           |                 |                   |         |                   |
| JP 2927530                                                                                                                                      | 7/1999           |                 |                   |         |                   |
| JP 2004/107556                                                                                                                                  | 4/2004           |                 |                   |         |                   |
| JP 2005/162968                                                                                                                                  | 6/2005           |                 |                   |         |                   |
| WO WO 2010/009036                                                                                                                               | 1/2010           |                 |                   |         |                   |
| OTHER PUBLICATIONS                                                                                                                              |                  |                 |                   |         |                   |
| Singapore Search Report issued from the Singapore Patent Office dated Jun. 30, 2014 in counterpart Singapore Patent Application No. 2012067781. |                  |                 |                   |         |                   |
| * cited by examiner                                                                                                                             |                  |                 |                   |         |                   |



## NATURAL GAS ENGINE LUBRICATING OIL COMPOSITIONS

### BACKGROUND OF THE INVENTION

#### 1. Technical Field

The present invention generally relates to a natural gas engine lubricating oil composition and a method for preventing or inhibiting exhaust valve seat recession in natural gas fueled internal combustion engines.

#### 2. Description of the Related Art

Natural gas fueled engines are engines that use natural gas as a fuel source. Lubricating oils with high resistance to oxidation, nitration and viscosity increase are generally preferred for lubricating oils used in natural gas engines because of the conditions related to this type of engine.

Natural gas has a higher specific heat content than liquid hydrocarbon fuels and therefore it will burn hotter than liquid hydrocarbon fuels under typical conditions. In addition, since it is already a gas, natural gas does not cool the intake air by evaporation as compared to liquid hydrocarbon fuel droplets. Furthermore, many natural gas fueled engines are run either at or near stoichiometric conditions, where less excess air is available to dilute and cool combustion gases. As a result, natural gas fueled engines generate higher combustion gas temperatures than engines burning liquid hydrocarbon fuels. In most cases, natural gas fueled engines are used continuously at 70 to 100% load, whereas an engine operating in vehicular service may only spend 50% of its time at full load.

This condition of running continuously near full load places severe demands on the lubricant. For example, by subjecting the lubricating to a sustained high temperature environment, the life of the lubricant is often limited by oil oxidation processes. Also, since the rate of formation of oxides of nitrogen (NO<sub>x</sub>) increases exponentially with temperature, natural gas fueled engines may generate NO<sub>x</sub> concentrations high enough to cause severe nitration of lubricating oil.

Good valve wear control is also important for keeping engine operating costs down and may be achieved by providing the proper amount and composition of ash. In addition, minimizing combustion chamber deposits and spark plug fouling are considerations in setting the ash content in these oils. Lubricating oil ash levels are limited, so detergents must be carefully selected to minimize piston deposits and ring sticking.

Valve wear resistance is important to the durability of natural gas fueled engines. In general, exhaust valve recession is wear which occurs at the valve and valve seat interface and is the most pronounced form of valve wear in natural gas fueled engines. When the valve is prevented from seating properly, it can cause engine roughness, poor fuel economy and excessive emissions. In order to correct excessive valve wear, a cylinder head overhaul is usually required. Although natural gas fueled engines typically use very hard corrosion-resistant material for the valve face and seat mating surface to give extended cylinder head life, it does not completely eliminate valve recession.

There is a difference in the lubricating oil requirements for natural gas fueled engines and engines that are fueled by liquid hydrocarbon fuels. The combustion of liquid hydrocarbon fuels such as diesel fuel often results in a small amount of incomplete combustion (e.g., exhaust particulates). In a liquid hydrocarbon fueled engine, these incombustibles provide a small but critical degree of lubrication to the exhaust valve/seat interface, thereby ensuring the durability of both cylinder heads and valves.

Natural gas fueled engines burn fuel that is introduced to the combustion chamber in the gaseous phase. The combustion of natural gas fuel is often very complete, with virtually no incombustible materials. This has a significant affect on the intake and exhaust valves because there is no fuel-derived lubricant such as liquid droplets or soot to aid in lubrication to the exhaust valve/seat interface in a natural gas fueled engine. Therefore, the durability of the cylinder head and valve is controlled by the ash content and other properties of the lubricating oil and its consumption rate to provide lubricant between the hot valve face and its mating seat. Too little ash or the wrong type can accelerate valve and seat wear, while too much ash may lead to valve guttering and subsequent valve torching. Too much ash can also lead to loss of compression or detonation from combustion chamber deposits. Consequently, gas engine builders frequently specify a narrow ash range that they have learned provides the optimum performance. Since most gas is low in sulfur, excess ash is generally not needed to address alkalinity requirements, and ash levels are largely optimized around the needs of the valves. There may be exceptions to this in cases where sour gas or landfill gas is used. The use of catalysts is becoming more prevalent as a means to meet stricter emission regulations. Limiting phosphorous content in the lubricating oil can prevent catalyst poisoning.

U.S. Pat. No. 3,798,163 ("the '163 patent") discloses a method for controlling or inhibiting exhaust valve recession in natural gas fueled internal combustion engines by maintaining a lubricating amount of a lubricating oil composition on the engine components of the internal combustion engine. The '163 patent further discloses that the lubricating oil composition contains (a) a major amount of an oil of lubricating viscosity, (b) at least one alkaline earth metal sulfonate in an amount sufficient to improve the detergency of the composition, and (c) at least one alkaline earth metal salt of a condensation product of (i) an alkylene polyamine, (ii) an aldehyde, and (iii) a substituted phenol, wherein the alkaline earth metal salt of the condensation product is present in an amount sufficient to inhibit the recession of the engine's exhaust valves into the engine cylinder head.

U.S. Pat. No. 5,726,133 ("the '133 patent") discloses a low ash gas engine oil comprising a major amount of a base oil of lubricating viscosity and a minor amount sufficient to contribute a sulfated ash content of about 0.1 to 0.6% ash by ASTM D 874 of an additive mixture comprising a mixture of detergents comprising at least one first alkali or alkaline earth metal salt or mixture thereof of low Total Base Number (TBN) of about 250 and less and at least one second alkali or alkaline earth metal salt or mixture thereof which is more neutral than the first low TBN salt. The '133 patent further discloses that the fully formulated gas engine oil can also typically contain other standard additives known to those skilled in the art, including anti-wear additives such as zinc dithiophosphates, dispersants, phenolic or aminic antioxidants, metal deactivators, pour point depressants, antifoaming agents, and viscosity index improvers.

U.S. Pat. No. 6,174,842 ("the '842 patent") discloses a lubricating composition containing (a) a major amount of lubricating oil, (b) an oil-soluble molybdenum compound substantially free of reactive sulfur, (c) an oil-soluble diarylamine and (d) an alkaline earth metal phenate. The '842 patent further discloses that the composition can further include a zinc dihydrocarbyl dithiophosphate as an anti-wear agent. In addition, Oil Blend 18 disclosed in Example 2 of the '842 patent contained an anti-wear agent and was evaluated for exhaust valve recession in a Cummins Natural Gas Engine test.

U.S. Patent Application Publication No. 20070129263 ("the '263 application") discloses a lubricating oil composition containing (a) a major amount of an oil of lubricating viscosity (b) one or more lithium-containing detergents (c) one or more detergents other than a lithium-containing detergent (d) one or more antioxidants (e) one or more dispersants and (f) one or more anti-wear agents, wherein the lubricating oil composition contains no more than 0.1 weight percent of lithium-containing detergents and no more than 0.12 weight percent phosphorus, and provided the lubricating oil composition does not contain a calcium-containing detergent. The '263 application further discloses that the lubricating oil composition is useful for reducing catalyst poisoning in exhaust after treatment in internal combustion engines such as diesel engines, gasoline engines and natural gas engines.

It is desirable to develop improved natural gas engine lubricating oil compositions which can prevent or inhibit exhaust valve recession in natural gas fueled internal combustion engines.

#### SUMMARY OF THE INVENTION

In accordance with one embodiment of the present invention, a natural gas engine lubricating oil composition is provided comprising (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents.

In accordance with a second embodiment of the present invention, a natural gas engine lubricating oil composition is provided comprising (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid as the only detergent in the natural gas engine lubricating oil composition, and (e) one or more antioxidants, wherein the natural gas engine lubricating oil composition contains no more than about 0.03 weight percent of phosphorus, based on the total weight of the natural gas engine lubricating oil composition.

In accordance with a third embodiment of the present invention, there is provided a method for preventing or inhibiting exhaust valve seat recession in a natural gas fueled engine, the method comprising lubricating the engine with a natural gas engine lubricating oil composition comprising (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents.

In accordance with a fourth embodiment of the present invention, there is provided a method for enhancing the life of an exhaust valve in a natural gas fueled engine as evidenced by protection or inhibition in exhaust valve seat recession in

the natural gas fueled engine, the method comprising lubricating the natural gas fueled engine with a natural gas engine lubricating oil composition comprising (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents.

In accordance with a fifth embodiment of the present invention, the use of a natural gas engine lubricating oil composition comprising (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents for the purpose of preventing or inhibiting exhaust valve seat recession in a natural gas fueled engine is provided.

By lubricating a natural gas fueled internal combustion engine with a natural gas engine lubricating oil composition comprising (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents, exhaust valve seat recession in the natural gas fueled engine is prevented or inhibited.

In addition, the natural gas engine lubricating oil composition of the present invention advantageously possesses improved or relatively comparable exhaust valve seat recession properties in a natural gas fueled engine as compared to a corresponding natural gas engine lubricating oil composition in which the one or more alkaline earth metal salts of an alkyl-substituted hydroxyaromatic carboxylic acid in the natural gas engine lubricating oil composition is replaced with an alkaline earth metal-containing phenate detergent.

#### BRIEF DESCRIPTION OF THE DRAWING

FIG. 1 is a bar graph comparing the exhaust valve recession wear rates for the lubricating oil composition of Example 1 versus the lubricating oil composition of Comparative Example A.

#### DETAILED DESCRIPTION OF THE PREFERRED EMBODIMENTS

To facilitate the understanding of the subject matter disclosed herein, a number of terms, abbreviations or other shorthand as used herein are defined below. Any term, abbreviation or shorthand not defined is understood to have the

ordinary meaning used by a skilled artisan contemporaneous with the submission of this application.

#### Definitions

The term "alkaline earth metal" refers to calcium, barium, magnesium, and strontium.

The term "alkali metal" refers to lithium, sodium, potassium, rubidium, and cesium.

The term "carboxylate" means an alkaline earth metal salts of an alkyl-substituted hydroxyaromatic carboxylic acid.

The term "phenate" means a salt of a phenol.

The present invention is directed to a natural gas engine lubricating oil composition containing (a) a major amount of an oil of lubricating viscosity, (b) one or more phosphorus-containing anti-wear additives, (c) one or more ashless dispersants, (d) one or more alkaline earth metal salts of an alkyl-substituted hydroxyaromatic carboxylic acid, and (e) one or more antioxidants, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents. The term "substantially free" as used herein shall be understood to mean only trace amounts, typically below 0.001 wt. %, based on the total weight of the natural gas engine lubricating oil composition, if any, of alkali metal-containing detergents in the natural gas engine lubricating oil composition.

In one embodiment, the natural gas engine lubricating oil compositions according to the present invention contain from about 0.005 to about 0.03 wt. % of phosphorus, based on the total weight of the natural gas engine lubricating oil composition.

In one embodiment, a natural gas engine lubricating oil composition according to the present invention will have a sulfated ash content of no more than about 1.25 wt. % as determined by ASTM D 874. In another embodiment, a natural gas engine lubricating oil composition according to the present invention will have a sulfated ash content of no more than about 0.3 wt. % as determined by ASTM D 874. In one embodiment, a natural gas engine lubricating oil composition according to the present invention for use in natural gas fueled engines has a sulfated ash content of about 0.1 wt. % to about 1.25 wt. % as determined by ASTM D 874. In another embodiment, a natural gas engine lubricating oil composition according to the present invention will have a sulfated ash content of about 0.12 wt. % to about 1.0 wt. % as determined by ASTM D 874. In another embodiment, a natural gas engine lubricating oil composition according to the present invention will have a sulfated ash content of about 0.15 wt. % to about 0.3 wt. % as determined by ASTM D 874. The lubricant ash advantageously acts as a solid lubricant to protect the valve/seat interface in place of naturally occurring exhaust particles in a hydrocarbon fueled engine.

In another embodiment, a natural gas engine lubricating oil composition according to the present invention contains relatively low levels of sulfur, i.e., not exceeding 0.7 wt. %, preferably not exceeding 0.5 wt. % and more preferably not exceeding 0.3 wt. %, based on the total weight of the natural gas engine lubricating oil composition.

The internal combustion engines to which the present invention is applicable may be characterized as those operated on, i.e., fueled by, natural gas and include internal combustion engines. Examples of such engines include four cycle

engines and the like. In one preferred embodiment, the internal combustion engine is a stationary engine used in, for example, well-head gas gathering, compression, and other gas pipeline services; electrical power generation (including co-generation); and irrigation.

The oil of lubricating viscosity for use in a natural gas engine lubricating oil compositions of this invention, also referred to as a base oil, is typically present in a major amount, e.g., an amount greater than 50 wt. %, preferably greater than 10 about 70 wt. %, more preferably from about 80 to about 99.5 wt. % and most preferably from about 85 to about 98 wt. %, based on the total weight of the composition. The expression "base oil" as used herein shall be understood to mean a base stock or blend of base stocks which is a lubricant component 15 that is produced by a single manufacturer to the same specifications (independent of feed source or manufacturer's location); that meets the same manufacturer's specification; and that is identified by a unique formula, product identification number, or both. The base oil for use herein can be any 20 presently known or later-discovered oil of lubricating viscosity used in formulating lubricating oil compositions for any and all such applications, e.g., engine oils, marine cylinder oils, functional fluids such as hydraulic oils, gear oils, transmission fluids, etc. Additionally, the base oils for use herein 25 can optionally contain viscosity index improvers, e.g., polymeric alkylmethacrylates; olefinic copolymers, e.g., an ethylene-propylene copolymer or a styrene-butadiene copolymer; and the like and mixtures thereof.

As one skilled in the art would readily appreciate, the 30 viscosity of the base oil is dependent upon the application. Accordingly, the viscosity of a base oil for use herein will ordinarily range from about 2 to about 2000 centistokes (cSt) at 100° Centigrade (C). Generally, individually the base oils used herein will have a kinematic viscosity range at 100° C. of 35 about 2 cSt to about 30 cSt. In one embodiment, the base oils used herein will have a kinematic viscosity range at 100° C. of about 5 cSt to about 20 cSt. In one embodiment, the base oils used herein will have a kinematic viscosity range at 100° C. of about 7 cSt to about 15 cSt. The base oil will be selected or 40 blended depending on the desired end use and the additives in the finished oil to give the desired grade of oil, e.g., a lubricating oil composition having an SAE Viscosity Grade of 0W, 0W-20, 0W-30, 0W-40, 0W-50, 0W-60, 5W, 5W-20, 5W-30, 5W-40, 5W-50, 5W-60, 10W, 10W-20, 10W-30, 10W-40, 45 10W-50, 15W, 15W-20, 15W-30, 15W-40, 30, 40 and the like.

Base stocks may be manufactured using a variety of different processes including, but not limited to, distillation, solvent refining, hydrogen processing, oligomerization, esterification, and rerefining. Rerefined stock shall be substantially free from materials introduced through manufacturing, contamination, or previous use. The base oil of the lubricating oil compositions of this invention may be any natural or synthetic lubricating base oil. Suitable hydrocarbon synthetic oils include, but are not limited to, oils prepared 50 from the polymerization of ethylene or from the polymerization of 1-olefins to provide polymers such as polyalphaolefin or PAO oils, or from hydrocarbon synthesis procedures using carbon monoxide and hydrogen gases such as in a Fischer-Tropsch process. For example, a suitable base oil is one that 55 comprises little, if any, heavy fraction; e.g., little, if any, lube oil fraction of viscosity 20 cSt or higher at 100° C.

The base oil may be derived from natural lubricating oils, synthetic lubricating oils or mixtures thereof. Suitable base oil includes base stocks obtained by isomerization of synthetic wax and slack wax, as well as hydrocracked base stocks produced by hydrocracking (rather than solvent extracting) 60 the aromatic and polar components of the crude. Suitable base

oils include those in all API categories I, II, III, IV and V as defined in API Publication 1509, 16<sup>th</sup> Edition, Addendum I, October, 2009. Group IV base oils are polyalphaolefins (PAO). Group V base oils include all other base oils not included in Group I, II, III, or IV. Although Group II, III and IV base oils are preferred for use in this invention, these base oils may be prepared by combining one or more of Group I, II, III, IV and V base stocks or base oils.

Useful natural oils include mineral lubricating oils such as, for example, liquid petroleum oils, solvent-treated or acid-treated mineral lubricating oils of the paraffinic, naphthenic or mixed paraffinic-naphthenic types, oils derived from coal or shale, animal oils, vegetable oils (e.g., rapeseed oils, castor oils and lard oil), and the like.

Useful synthetic lubricating oils include, but are not limited to, hydrocarbon oils and halo-substituted hydrocarbon oils such as polymerized and interpolymerized olefins, e.g., polybutylenes, polypropylenes, propylene-isobutylene copolymers, chlorinated polybutylenes, poly(1-hexenes), poly(1-octenes), poly(1-decenes), and the like and mixtures thereof; alkylbenzenes such as dodecylbenzenes, tetradecylbenzenes, dinonylbenzenes, di(2-ethylhexyl)-benzenes, and the like; polyphenyls such as biphenyls, terphenyls, alkylated polyphenyls, and the like; alkylated diphenyl ethers and alkylated diphenyl sulfides and the derivative, analogs and homologs thereof and the like.

Other useful synthetic lubricating oils include, but are not limited to, oils made by polymerizing olefins of less than 5 carbon atoms such as ethylene, propylene, butylenes, isobutene, pentene, and mixtures thereof. Methods of preparing such polymer oils are well known to those skilled in the art.

Additional useful synthetic hydrocarbon oils include liquid polymers of alpha olefins having the proper viscosity. Especially useful synthetic hydrocarbon oils are the hydrogenated liquid oligomers of C<sub>6</sub> to C<sub>12</sub> alpha olefins such as, for example, 1-decene trimer.

Another class of useful synthetic lubricating oils includes, but are not limited to, alkylene oxide polymers, i.e., homopolymers, interpolymers, and derivatives thereof where the terminal hydroxyl groups have been modified by, for example, esterification or etherification. These oils are exemplified by the oils prepared through polymerization of ethylene oxide or propylene oxide, the alkyl and phenyl ethers of these polyoxyalkylene polymers (e.g., methyl poly propylene glycol ether having an average molecular weight of 1,000, diphenyl ether of polyethylene glycol having a molecular weight of 500-1000, diethyl ether of polypropylene glycol having a molecular weight of 1,000-1,500, etc.) or mono- and polycarboxylic esters thereof such as, for example, the acetic esters, mixed C<sub>3</sub>-C<sub>8</sub> fatty acid esters, or the C<sub>13</sub> oxo acid diester of tetraethylene glycol.

Yet another class of useful synthetic lubricating oils include, but are not limited to, the esters of dicarboxylic acids e.g., phthalic acid, succinic acid, alkyl succinic acids, alkenyl succinic acids, maleic acid, azelaic acid, suberic acid, sebacic acid, fumaric acid, adipic acid, linoleic acid dimer, malonic acids, alkyl malonic acids, alkenyl malonic acids, etc., with a variety of alcohols, e.g., butyl alcohol, hexyl alcohol, dodecyl alcohol, 2-ethylhexyl alcohol, ethylene glycol, diethylene glycol monoether, propylene glycol, etc. Specific examples of these esters include dibutyl adipate, di(2-ethylhexyl)sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, the complex ester formed by reacting one mole of

sebacic acid with two moles of tetraethylene glycol and two moles of 2-ethylhexanoic acid and the like.

Esters useful as synthetic oils also include, but are not limited to, those made from carboxylic acids having from about 5 to about 12 carbon atoms with alcohols, e.g., methanol, ethanol, etc., polyols and polyol ethers such as neopentyl glycol, trimethylol propane, pentaerythritol, dipentaerythritol, tripentaerythritol, and the like.

Silicon-based oils such as, for example, polyalkyl-, polyaryl-, polyalkoxy- or polyaryloxy-siloxane oils and silicate oils, comprise another useful class of synthetic lubricating oils. Specific examples of these include, but are not limited to, tetraethyl silicate, tetra-isopropyl silicate, tetra-(2-ethylhexyl) silicate, tetra-(4-methyl-hexyl) silicate, tetra-(p-tert-butylphenyl) silicate, hexyl-(4-methyl-2-pentoxy) disiloxane, poly(methyl) siloxanes, poly(methylphenyl) siloxanes, and the like. Still yet other useful synthetic lubricating oils include, but are not limited to, liquid esters of phosphorous containing acids, e.g., tricresyl phosphate, trioctyl phosphate, diethyl ester of decane phosphonic acid, etc., polymeric tetrahydrofurans and the like.

The lubricating oil may be derived from unrefined, refined and rerefined oils, either natural, synthetic or mixtures of two or more of any of these of the type disclosed hereinabove.

Unrefined oils are those obtained directly from a natural or synthetic source (e.g., coal, shale, or tar sands bitumen) without further purification or treatment. Examples of unrefined oils include, but are not limited to, a shale oil obtained directly from retorting operations, a petroleum oil obtained directly from distillation or an ester oil obtained directly from an esterification process, each of which is then used without further treatment. Refined oils are similar to the unrefined oils except they have been further treated in one or more purification steps to improve one or more properties. These purification techniques are known to those of skill in the art and include, for example, solvent extractions, secondary distillation, acid or base extraction, filtration, percolation, hydrotreating, dewaxing, etc. Rerefined oils are obtained by treating used oils in processes similar to those used to obtain refined oils. Such rerefined oils are also known as reclaimed or reprocessed oils and often are additionally processed by techniques directed to removal of spent additives and oil breakdown products.

Lubricating oil base stocks derived from the hydroisomerization of wax may also be used, either alone or in combination with the aforesaid natural and/or synthetic base stocks. Such wax isomerate oil is produced by the hydroisomerization of natural or synthetic waxes or mixtures thereof over a hydroisomerization catalyst.

Natural waxes are typically the slack waxes recovered by the solvent dewaxing of mineral oils; synthetic waxes are typically the wax produced by the Fischer-Tropsch process. Examples of useful oils of lubricating viscosity include HVI and XHVI basestocks, such isomerized wax base oils and UCBO (Unconventional Base Oils) base oils.

The natural gas engine lubricating oil compositions of the present invention will also contain one or more phosphorus-containing anti-wear additives, wherein the natural gas engine lubricating oil composition contains no more than about 0.03 weight percent of phosphorus, based on the total weight of the natural gas engine lubricating oil composition. Suitable phosphorus-containing anti-wear additives include, but are not limited to, hydrocarbyl phosphites such as trialkyl phosphites aryl-containing phosphites, e.g., triaryl phosphites, and the like; hydrocarbyl phosphates such as trialkyl phosphates, aryl-containing phosphates, e.g., triaryl phosphates, alkyl diaryl phosphates and the like and mixtures

thereof. In one embodiment, at least two phosphorus-containing anti-wear additives are used in the natural gas engine lubricating oil composition.

Representative examples of trialkyl phosphites include, but are not limited to, tributyl phosphite, trihexyl phosphite, trioctyl phosphite, tridecyl phosphite, trilauryl phosphite, trioleyl phosphite and the like. Representative examples of aryl-containing phosphites include triaryl phosphites such as triphenyl phosphite, tricresylphosphite and the like.

Representative examples of trialkyl phosphates include, but are not limited to, tributyl phosphate, trihexyl phosphate, trioctyl phosphate, tridecyl phosphate, trilauryl phosphate, trioleyl phosphate and the like. Representative examples of aryl-containing phosphates include, but are not limited to, butyl diphenyl phosphate, dibutyl phenyl phosphate, t-butylphenyl diphenyl phosphate, bis(t-butylphenyl) phenyl phosphate, tri(t-butylphenyl)phosphate, triphenyl phosphate, and propylated triphenyl phosphate, and the like and mixtures thereof.

In one embodiment, the one or more phosphorus-containing anti-wear additives includes a zinc dialkyldithiophosphate (Zn-DTP, primary alkyl type & secondary alkyl type).

In general, the one or more phosphorus-containing anti-wear additives are collectively present in the natural gas engine lubricating oil composition in an amount ranging from about 0.25 to about 1.5 wt. %, based on the total weight of the natural gas engine lubricating oil composition.

The one or more ashless dispersant compounds (c) employed in the natural gas engine lubricating oil composition of the present invention are generally used to maintain in suspension insoluble materials resulting from oxidation during use, thus preventing sludge flocculation and precipitation or deposition on metal parts. Nitrogen-containing ashless (metal-free) dispersants are basic, and contribute to the base number or BN (as can be measured by ASTM D 2896) of a lubricating oil composition to which they are added, without introducing additional sulfated ash. The term "Base Number" or "BN" as used herein refers to the amount of base equivalent to milligrams of KOH in one gram of sample. Thus, higher BN numbers reflect more alkaline products, and therefore a greater alkalinity. BN was determined using ASTM D 2896 test. An ashless dispersant generally comprises an oil soluble polymeric hydrocarbon backbone having functional groups that are capable of associating with particles to be dispersed. Many types of ashless dispersants are known in the art.

Representative examples of ashless dispersants include, but are not limited to, amines, alcohols, amides, or ester polar moieties attached to the polymer backbones via bridging groups. An ashless dispersant of the present invention may be, for example, selected from oil soluble salts, esters, amino-esters, amides, imides, and oxazolines of long chain hydrocarbon substituted mono and dicarboxylic acids or their anhydrides; thiocarboxylate derivatives of long chain hydrocarbons, long chain aliphatic hydrocarbons having a polyamine attached directly thereto; and Mannich condensation products formed by condensing a long chain substituted phenol with formaldehyde and polyalkylene polyamine.

Carboxylic dispersants are reaction products of carboxylic acylating agents (acids, anhydrides, esters, etc.) comprising at least about 34 and preferably at least about 54 carbon atoms with nitrogen containing compounds (such as amines), organic hydroxy compounds (such as aliphatic compounds including monohydric and polyhydric alcohols, or aromatic compounds including phenols and naphthols), and/or basic inorganic materials. These reaction products include imides, amides, and esters.

Succinimide dispersants are a type of carboxylic dispersant. They are produced by reacting hydrocarbyl-substituted succinic acylating agent with organic hydroxy compounds, or with amines comprising at least one hydrogen atom attached to a nitrogen atom, or with a mixture of the hydroxy compounds and amines. The term "succinic acylating agent" refers to a hydrocarbon-substituted succinic acid or a succinic acid-producing compound, the latter encompasses the acid itself. Such materials typically include hydrocarbyl-substituted succinic acids, anhydrides, esters (including half esters) and halides.

Succinic-based dispersants have a wide variety of chemical structures. One class of succinic-based dispersants may be represented by the formula:



wherein each R<sup>1</sup> is independently a hydrocarbyl group, such as a polyolefin-derived group. Typically the hydrocarbyl group is an alkyl group, such as a polyisobutyl group. Alternatively expressed, the R<sup>1</sup> groups can contain about 40 to about 500 carbon atoms, and these atoms may be present in aliphatic forms. R<sup>2</sup> is an alkylene group, commonly an ethylene (C<sub>2</sub>H<sub>4</sub>) group. Examples of succinimide dispersants include those described in, for example, U.S. Pat. Nos. 3,172,892, 4,234,435 and 6,165,235.

The polyalkenes from which the substituent groups are derived are typically homopolymers and interpolymers of polymerizable olefin monomers of 2 to about 16 carbon atoms, and usually 2 to 6 carbon atoms. The amines which are reacted with the succinic acylating agents to form the carboxylic dispersant composition can be monoamines or polyamines.

Succinimide dispersants are referred to as such since they normally contain nitrogen largely in the form of imide functionality, although the amide functionality may be in the form of amine salts, amides, imidazolines as well as mixtures thereof. To prepare a succinimide dispersant, one or more succinic acid-producing compounds and one or more amines are heated and typically water is removed, optionally in the presence of a substantially inert organic liquid solvent/diluent. The reaction temperature can range from about 80° C. up to the decomposition temperature of the mixture or the product, which typically falls between about 100° C. to about 300° C. Additional details and examples of procedures for preparing the succinimide dispersants of the present invention include those described in, for example, U.S. Pat. Nos. 3,172,892, 3,219,666, 3,272,746, 4,234,435, 6,165,235 and 6,440,905.

Suitable ashless dispersants may also include amine dispersants, which are reaction products of relatively high molecular weight aliphatic halides and amines, preferably polyalkylene polyamines. Examples of such amine dispersants include those described in, for example, U.S. Pat. Nos. 3,275,554, 3,438,757, 3,454,555 and 3,565,804.

Suitable ashless dispersants may further include "Mannich dispersants," which are reaction products of alkyl phenols in which the alkyl group contains at least about 30 carbon atoms with aldehydes (especially formaldehyde) and amines (especially polyalkylene polyamines). Examples of such dispers-

## 11

ants include those described in, for example, U.S. Pat. Nos. 3,036,003, 3,586,629, 3,591,598 and 3,980,569.

Suitable ashless dispersants may also be post-treated ashless dispersants such as post-treated succinimides, e.g., post-treatment processes involving borate or ethylene carbonate as disclosed in, for example, U.S. Pat. Nos. 4,612,132 and 4,746,446; and the like as well as other post-treatment processes. The carbonate-treated alkenyl succinimide is a polybutene succinimide derived from polybutenes having a molecular weight of about 450 to about 3000, preferably from about 900 to about 2500, more preferably from about 1300 to about 2400, and most preferably from about 2000 to about 2400, as well as mixtures of these molecular weights. Preferably, it is prepared by reacting, under reactive conditions, a mixture of a polybutene succinic acid derivative, an unsaturated acidic reagent copolymer of an unsaturated acidic reagent and an olefin, and a polyamine, such as disclosed in U.S. Pat. No. 5,716,912, the contents of which are incorporated herein by reference.

Suitable ashless dispersants may also be polymeric, which are interpolymers of oil-solubilizing monomers such as decyl methacrylate, vinyl decyl ether and high molecular weight olefins with monomers containing polar substitutes. Examples of polymeric dispersants include those described in, for example, U.S. Pat. Nos. 3,329,658; 3,449,250 and 3,666,730.

In a preferred embodiment of the present invention, an ashless dispersant for use in the natural gas engine lubricating oil composition is a bis-succinimide derived from a polyisobutetyl group having a number average molecular weight of about 700 to about 2300. The dispersant(s) for use in the lubricating oil compositions of the present invention are preferably non-polymeric (e.g., are mono- or bis-succinimides).

Generally, the one or more ashless dispersants are present in the natural gas engine lubricating oil composition in an amount ranging from about 1 to about 8 wt. %, based on the total weight of the natural gas engine lubricating oil composition. In one embodiment, the one or more ashless dispersants are present in the natural gas engine lubricating oil composition in an amount ranging from about 1.5 to about 6 wt. %, based on the total weight of the natural gas engine lubricating oil composition.

The one or more alkaline earth metal salts of an alkyl-substituted hydroxyaromatic carboxylic acid (d) employed in the natural gas engine lubricating oil composition of the present invention function both as a detergent to reduce or remove deposits and as an acid neutralizer or rust inhibitor, thereby reducing wear and corrosion and extending engine life. Detergents generally comprise a polar head with long hydrophobic tail, with the polar head comprising a metal salt of an acid organic compound.

Suitable hydroxyaromatic compounds include mono-nuclear monohydroxy and polyhydroxy aromatic hydrocarbons having 1 to 4, and preferably 1 to 3, hydroxyl groups. Suitable hydroxyaromatic compounds include phenol, catechol, resorcinol, hydroquinone, pyrogallol, cresol, and the like. The preferred hydroxyaromatic compound is phenol.

The alkyl substituted moiety of the alkaline earth metal salt of an alkyl-substituted hydroxyaromatic carboxylic acid is derived from an alpha olefin having from about 10 to about 80 carbon atoms. The olefins employed may be linear, isomerized linear, branched or partially branched linear. The olefin may be a mixture of linear olefins, a mixture of isomerized linear olefins, a mixture of branched olefins, a mixture of partially branched linear or a mixture of any of the foregoing.

In one embodiment, the mixture of linear olefins that may be used is a mixture of normal alpha olefins selected from

## 12

olefins having from about 12 to about 30 carbon atoms per molecule. In one embodiment, the normal alpha olefins are isomerized using at least one of a solid or liquid catalyst.

In another embodiment, the olefins are a branched olefinic propylene oligomer or mixture thereof having from about 20 to about 80 carbon atoms, i.e., branched chain olefins derived from the polymerization of propylene. The olefins may also be substituted with other functional groups, such as hydroxy groups, carboxylic acid groups, heteroatoms, and the like. In one embodiment, the branched olefinic propylene oligomer or mixtures thereof have from about 20 to about 60 carbon atoms. In one embodiment, the branched olefinic propylene oligomer or mixtures thereof have from about 20 to about 40 carbon atoms.

In one embodiment, at least about 75 mole % (e.g., at least about 80 mole %, at least about 85 mole %, at least about 90 mole %, at least about 95 mole %, or at least about 99 mole %) of the alkyl groups contained within the alkaline earth metal salt of an alkyl-substituted hydroxyaromatic carboxylic acid such as the alkyl groups of an alkaline earth metal salt of an alkyl-substituted hydroxybenzoic acid detergent are a C<sub>20</sub> or higher. In another embodiment, the alkaline earth metal salt of an alkyl-substituted hydroxyaromatic carboxylic acid is an alkaline earth metal salt of an alkyl-substituted hydroxybenzoic acid that is derived from an alkyl-substituted hydroxybenzoic acid in which the alkyl groups are the residue of normal alpha-olefins containing at least 75 mole % C<sub>20</sub> or higher normal alpha-olefins.

In another embodiment, at least about 50 mole % (e.g., at least about 60 mole %, at least about 70 mole %, at least about 80 mole %, at least about 85 mole %, at least about 90 mole %, at least about 95 mole %, or at least about 99 mole %) of the alkyl groups contained within the alkaline earth metal salt of an alkyl-substituted hydroxyaromatic carboxylic acid such as the alkyl groups of an alkaline earth metal salt of an alkyl-substituted hydroxybenzoic acid are about C<sub>14</sub> to about C<sub>18</sub>.

The alkaline earth metals useful in making the one or more alkaline earth metal salts of an alkyl-substituted hydroxyaromatic carboxylic acid include, but are not limited to, magnesium, calcium, strontium, barium and the like. In one embodiment, the alkaline earth metal compound is calcium.

The resulting alkaline earth metal salt of an alkyl-substituted hydroxyaromatic carboxylic acid will be a mixture of ortho and para isomers. In one embodiment, the product will contain about 1 to 99% ortho isomer and 99 to 1% para isomer. In another embodiment, the product will contain about 5 to 70% ortho and 95 to 30% para isomer.

The alkaline earth metal salts of an alkyl-substituted hydroxyaromatic carboxylic acid can be overbased or neutral. Generally, an overbased alkaline earth metal salt of an alkyl-substituted hydroxyaromatic carboxylic acid is one in which the BN of the alkaline earth metal salts of an alkyl-substituted hydroxyaromatic carboxylic acid has been increased by a process such as the addition of a base source (e.g., lime) and an acidic overbasing compound (e.g., carbon dioxide).

Overbased salts suitable for use in the natural gas engine lubricating oil compositions of the present invention may be low overbased, e.g., an overbased salt having a BN below about 100. In one embodiment, the BN of a low overbased salt may be from about 5 to about 50. In another embodiment, the BN of a low overbased salt may be from about 10 to about 30. In yet another embodiment, the BN of a low overbased salt may be from about 15 to about 20.

Overbased detergents suitable for use in the natural gas engine lubricating oil compositions of the present invention may be medium overbased, e.g., an overbased salt having a BN from about 100 to about 250. In one embodiment, the BN

of a medium overbased salt may be from about 100 to about 200. In another embodiment, the BN of a medium overbased salt may be from about 125 to about 175.

Overbased detergents suitable for use in the natural gas engine lubricating oil compositions of the present invention may be high overbased, e.g., an overbased salt having a BN above about 250. In one embodiment, the BN of a high overbased salt may be from about 250 to about 450.

The natural gas engine lubricating oil compositions according to the present invention may contain more than one overbased salt, which may be all low BN salts, all medium BN salts, all high BN salts and mixtures thereof.

Generally, the one or more alkaline earth metal salts of an alkyl-substituted hydroxyaromatic carboxylic acid are present in the natural gas engine lubricating oil composition in an amount ranging from about 0.5 to about 2.5 wt. %, based on the total weight of the natural gas engine lubricating oil composition. In another embodiment, the one or more alkaline earth metal salts of an alkyl-substituted hydroxyaromatic carboxylic acid are present in the natural gas engine lubricating oil composition in an amount ranging from about 1.0 to about 2.0 wt. %, based on the total weight of the natural gas engine lubricating oil composition.

The one or more antioxidant compounds (e) employed in the natural gas engine lubricating oil composition of the present invention reduce the tendency of base stocks to deteriorate in service, which deterioration can be evidenced by the products of oxidation such as sludge and varnish-like deposits on the metal surfaces and by viscosity growth. Such oxidation inhibitors include hindered phenols, ashless oil soluble phenates and sulfurized phenates, diphenylamines, alkyl-substituted phenyl and naphthylamines and the like and mixtures thereof. Diphenyamine-type oxidation inhibitors include, but are not limited to, alkylated diphenylamine, phenyl- $\alpha$ -naphthylamine, and alkylated- $\alpha$ -naphthylamine.

In one embodiment, an antioxidant compound for use herein can be one or more hindered phenols having the general formula:



wherein R is a C<sub>1</sub> to C<sub>30</sub> hydrocarbyl group including by way of example, a substituted or unsubstituted alkyl group, substituted or unsubstituted cycloalkyl group, substituted or unsubstituted aryl group, substituted or unsubstituted heterocyclic group and the like. A representative example of a hindered phenol is 3,5-di-t-butyl 4-hydroxy phenol propionate. The hindered phenol, 3,5-di-t-butyl 4-hydroxy phenol propionate may be available commercially from, for example, Ciba Specialty Chemicals (Terrytown, N.Y.) as IRGANOX L135®, Crompton Corporation (Middlebury, Conn.) as Naugard® PS-48. In one embodiment, a hindered phenol is a liquid hindered phenol.

Generally, the one or more antioxidant compounds are present in the natural gas engine lubricating oil composition in an amount ranging from about 0.1 to about 5 wt. %, based on the total weight of the natural gas engine lubricating oil composition. In one embodiment, the one or more antioxidant

compounds are present in the natural gas engine lubricating oil composition in an amount ranging from about 0.2 to about 4 wt. %, based on the total weight of the natural gas engine lubricating oil composition.

The natural gas engine lubricating oil compositions of the present invention can be conveniently prepared by simply blending or mixing the additives with the oil of lubricating viscosity. The additives may also be preblended as a concentrate, as discussed hereinbelow, in the appropriate ratios to facilitate blending of a lubricating composition containing the desired concentration of additives. The additive package is blended with the base oil using a concentration at which they are both soluble in the oil and compatible with other additives in the desired finished lubricating oil. Compatibility in this instance generally means that the present compounds as well as being oil soluble in the applicable treat rate also do not cause other additives to precipitate under normal conditions. Suitable oil solubility/compatibility ranges for a given compound of lubricating oil formulation can be determined by those having ordinary skill in the art using routine solubility testing procedures. For example, precipitation from a formulated lubricating oil composition at ambient conditions (about 20° C. to 25° C.) can be measured by either actual precipitation from the oil composition or the formulation of a "cloudy" solution which evidences formation of insoluble wax particles.

In one embodiment, the natural gas engine lubricating oil compositions described herein can be substantially free of any alkaline earth metal salts of a condensation product of an alkylene polyamine, an aldehyde and a substituted phenol. In one embodiment, the lubricating oil compositions are also substantially free of any molybdenum-containing compounds. The alkylene polyamines of the condensation product can the following structure NH<sub>2</sub>[R(R)—NH]<sub>n</sub>H wherein R is an alkylene radical containing from about 2 about 6 carbon atoms, and n is an integer from 1 to about 10. Typical alkylene polyamines include diethylenetriamine, triethylenetetramine, tetraethylenepentamine and the like. The aldehydes are generally aliphatic aldehydes which contain from one to about 3 carbon atoms per molecule. The substituted phenols are the alkylated monohydric phenols having at least one alkyl group of sufficient length to impart oil-solubility to the condensation products. Representative alkyl phenols are those in which the alkyl group contains from about 4 to about 24 carbon atoms, and preferably those having from about 8 to about 24 carbon atoms, such as, for example, n-amyl phenol, diethylphenol, octyl phenol, nonyl phenol, p-ter-octyl phenol, a mixture of phenols, wax alkylated phenols and the like.

In one embodiment, the natural gas engine lubricating oil compositions of the present invention will contain sulfurized isobutylene. Sulfurized isobutylene is known by those skilled in the art to be an extreme pressure agent, effective in preventing wear in high pressure environments such as gear lubrication. Sulfurized isobutylene comprises a long chain hydrocarbon that is reacted with a various sulfur compounds that are incorporated into the chain. This provides an oil soluble compound that is effective in providing extreme pressure (EP) protection. Sulfurized isobutylene for use in certain embodiments of this invention may include one or more of sulfurized isobutylenes such as Mobilad C-100 and R. T. Vanderbilt Vanlube SB.

Generally, the natural gas engine lubricating oil compositions of this invention will contain from about 0.01 wt. % to about 0.5 wt. % sulfurized isobutylene. In another embodiment, the natural gas engine lubricating oil compositions of this invention will contain from about 0.02 wt. % to about 0.45 wt. % sulfurized isobutylene.

## 15

The natural gas engine lubricating oil compositions may also contain other conventional additives for imparting auxiliary functions to give a finished natural gas engine lubricating oil composition in which these additives are dispersed or dissolved. For example, the natural gas engine lubricating oil compositions may be blended with rust inhibitors, dehazing agents, demulsifying agents, metal deactivating agents, friction modifiers, pour point depressants, antifoaming agents, co-solvents, package compatibilisers, corrosion-inhibitors, dyes, extreme pressure agents and the like and mixtures thereof. A variety of the additives are known and commercially available. These additives, or their analogous compounds, can be employed for the preparation of the natural gas engine lubricating oil compositions of the invention by the usual blending procedures.

Examples of rust inhibitors include, but are not limited to, nonionic polyoxyalkylene agents, e.g., polyoxyethylene lauryl ether, polyoxyethylene higher alcohol ether, polyoxyethylene nonylphenyl ether, polyoxyethylene octylphenyl ether, polyoxyethylene octyl stearyl ether, polyoxyethylene oleyl ether, polyoxyethylene sorbitol monostearate, polyoxyethylene sorbitol monooleate, and polyethylene glycol monooleate; stearic acid and other fatty acids; dicarboxylic acids; metal soaps; fatty acid amine salts; metal salts of heavy sulfonic acid; partial carboxylic acid ester of polyhydric alcohol; phosphoric esters; (short-chain) alkenyl succinic acids; partial esters thereof and nitrogen-containing derivatives thereof; synthetic alkylsulfonates, e.g., metal dinonylnaphthalene sulfonates; and the like and mixtures thereof.

Examples of friction modifiers include, but are not limited to, alkoxylated fatty amines; borated fatty epoxides; fatty phosphites, fatty epoxides, fatty amines, borated alkoxylated fatty amines, metal salts of fatty acids, fatty acid amides, glycerol esters, borated glycerol esters; and fatty imidazolines as disclosed in U.S. Pat. No. 6,372,696, the contents of which are incorporated by reference herein; friction modifiers obtained from a reaction product of a C<sub>4</sub> to C<sub>75</sub>, preferably a C<sub>6</sub> to C<sub>24</sub>, and most preferably a C<sub>6</sub> to C<sub>20</sub>, fatty acid ester and a nitrogen-containing compound selected from the group consisting of ammonia, and an alkanolamine and the like and mixtures thereof.

Examples of antifoaming agents include, but are not limited to, polymers of alkyl methacrylate; polymers of dimethylsilicone and the like and mixtures thereof.

Examples of a pour point depressant include, but are not limited to, polymethacrylates, alkyl acrylate polymers, alkyl methacrylate polymers, di(tetra-paraffin phenol)phthalate, condensates of tetra-paraffin phenol, condensates of a chlorinated paraffin with naphthalene and combinations thereof. In one embodiment, a pour point depressant comprises an ethylene-vinyl acetate copolymer, a condensate of chlorinated paraffin and phenol, polyalkyl styrene and the like and combinations thereof. The amount of the pour point depressant may vary from about 0.01 wt. % to about 10 wt. %.

Examples of a demulsifier include, but are not limited to, anionic surfactants (e.g., alkyl-naphthalene sulfonates, alkyl benzene sulfonates and the like), nonionic alkoxylated alkylphenol resins, polymers of alkylene oxides (e.g., polyethylene oxide, polypropylene oxide, block copolymers of ethylene oxide, propylene oxide and the like), esters of oil soluble acids, polyoxyethylene sorbitan ester and the like and combinations thereof. The amount of the demulsifier may vary from about 0.01 wt. % to about 10 wt. %.

Examples of a corrosion inhibitor include, but are not limited to, half esters or amides of dodecylsuccinic acid, phosphate esters, thiophosphates, alkyl imidazolines, sarcosines

## 16

and the like and combinations thereof. The amount of the corrosion inhibitor may vary from about 0.01 wt. % to about 5 wt. %.

Examples of an extreme pressure agent include, but are not limited to, sulfurized animal or vegetable fats or oils, sulfurized animal or vegetable fatty acid esters, fully or partially esterified esters of trivalent or pentavalent acids of phosphorus, sulfurized olefins, dihydrocarbyl polysulfides, sulfurized Diels-Alder adducts, sulfurized dicyclopentadiene, sulfurized or co-sulfurized mixtures of fatty acid esters and monounsaturated olefins, co-sulfurized blends of fatty acid, fatty acid ester and alpha-olefin, functionally-substituted dihydrocarbyl polysulfides, thia-aldehydes, thia-ketones, epithio compounds, sulfur-containing acetal derivatives, co-sulfurized blends of terpene and acyclic olefins, and polysulfide olefin products, amine salts of phosphoric acid esters or thiophosphoric acid esters and the like and combinations thereof. The amount of the extreme pressure agent may vary from about 0.01 wt. % to about 5 wt. %.

Each of the foregoing additives, when used, is used at a functionally effective amount to impart the desired properties to the lubricant. Thus, for example, if an additive is a friction modifier, a functionally effective amount of this friction modifier would be an amount sufficient to impart the desired friction modifying characteristics to the lubricant. Generally, the concentration of each of these additives, when used, ranges from about 0.001% to about 20% by weight, and in one embodiment about 0.01% to about 10% by weight based on the total weight of the natural gas engine lubricating oil composition.

If desired, the lubricating oil additives may be provided as an additive package or concentrate in which the additives are incorporated into a substantially inert, normally liquid organic diluent such as, for example, mineral oil, naphtha, benzene, toluene or xylene to form an additive concentrate. These concentrates usually contain from about 20% to about 80% by weight of such diluent. Typically, a neutral oil having a viscosity of about 4 to about 8.5 cSt at 100° C. and preferably about 4 to about 6 cSt at 100° C. will be used as the diluent, though synthetic oils, as well as other organic liquids which are compatible with the additives and finished lubricating oil can also be used. The additive package will typically contain the additives, referred to above, in the desired amounts and ratios to facilitate direct combination with the requisite amount of base oil.

The following non-limiting examples are illustrative of the present invention.

## EXAMPLE 1

A natural gas engine lubricating oil composition was formed containing 1.135 wt. % of a bis-succinimide (derived from a 1300 MW polyisobutylene succinic anhydride (PIBSA)) and a mixture of heavy polyamine and diethylenetriamine, 1.865 wt. % of a bis-succinimide (derived from a 950 MW polyisobutylene succinic anhydride (PIBSA)) and a mixture of heavy polyamine and diethylenetriamine, 1.26 wt. % of a calcium carboxylate which is the calcium salt of an alkyl-substituted hydroxybenzoic acid (150 BN), 1.25 wt. % of a hindered phenol antioxidant, 0.14 wt. % of a sulfurized isobutylene, 0.05 copper deactivator, 0.19 wt. % of a primary zinc alkyl dithiophosphate, 0.02 wt. % foam inhibitor and the balance being a Group II base oil.

The natural gas engine lubricating oil composition had a sulfated ash content of 0.25 wt. % as determined by ASTM D 874 and a phosphorus content of 0.014 wt. %.

## COMPARATIVE EXAMPLE A

A natural gas engine lubricating oil composition was formed containing 1.135 wt. % of a bis-succinimide (derived from a 1300 MW polyisobutylene succinic anhydride (PIBSA)) and a mixture of heavy polyamine and diethylenetriamine, 1.865 wt. % of a bis-succinimide (derived from a 950 MW polyisobutylene succinic anhydride (PIBSA)) and a mixture of heavy polyamine and diethylenetriamine, 1.52 wt. % of a sulfurized calcium phenate (114 BN), 1.25 wt. % of a hindered phenol antioxidant, 0.14 wt. % of a sulfurized isobutylene, 0.05 copper deactivator, 0.19 wt. % of a primary zinc alkyl dithiophosphate, 0.02 wt. % foam inhibitor and the balance being a Group II base oil.

The natural gas engine lubricating oil composition had a sulfated ash content of 0.25 wt. % as determined by ASTM D 874 and a phosphorus content of 0.014 wt. %.

## Testing

A 6-cylinder Waukesha F11 GSID engine was instrumented in order to obtain dynamic voltage measurements from 12 valves—6 intake and 6 exhaust valves. The tests were run for 400 hours on the lubricating oil compositions of Example 1 and Comparative Example A and the average valve recession wear rates of an oil were calculated by a linear fit based on the last 300-hours of data from each test and reported on a wear rate per 1000 hours. The maximum valve recession wear rate allowed by the original equipment manufacturer (OEM) is 0.00020 inches/1000 hours. As shown in FIG. 1, the lubricating oil composition of Example 1 containing a calcium carboxylate detergent showed significantly improved valve recession (-0.00019 inches) over the lubricating oil composition of Comparative Example A containing a calcium phenate detergent (0.00065 inches). This represents a difference of 0.00084 inches per 1000 hours. A difference of at least 0.000416 is considered to be significantly different at 95% confidence. Accordingly, the use of a carboxylate detergent resulted in slight valve growth; hence the reason for a negative valve recession wear rate.

It will be understood that various modifications may be made to the embodiments disclosed herein. Therefore the above description should not be construed as limiting, but merely as exemplifications of preferred embodiments. For example, the functions described above and implemented as the best mode for operating the present invention are for illustration purposes only. Other arrangements and methods may be implemented by those skilled in the art without departing from the scope and spirit of this invention. Moreover, those skilled in the art will envision other modifications within the scope and spirit of the claims appended hereto.

## What is claimed is:

1. A method for preventing or inhibiting exhaust valve seat recession in a natural gas fueled engine, the method comprising lubricating a natural gas fueled engine in need of exhaust valve seat recession prevention or inhibition with a natural gas engine lubricating oil composition comprising (a) a major amount of an oil of lubricating viscosity; (b) one or more phosphorus-containing anti-wear additives comprising a primary zinc alkylidithiophosphate, (c) about 1 wt. % to about 8 wt. %, based on the total weight of the natural gas engine lubricating oil composition, of one or more ashless dispersants comprising a bisuccinimide, (d) about 0.5 wt. % to about 2.5 wt. %, based on the total weight of the natural gas engine lubricating oil composition, of one or more alkaline earth metal salts of an alkyl-substituted hydroxyaromatic carboxylic acid having a total base number of from about 100 to about 250, wherein the one or more alkaline earth metal salts of alkyl-substituted hydroxyaromatic carboxylic acid are one or more calcium salts of an alkyl-substituted hydroxybenzoic acid and (e) about 0.1 wt. % to about 5 wt. %, based on the total weight of the natural gas engine lubricating oil composition, of one or more antioxidants comprising a hindered phenol compound, wherein the natural gas engine lubricating oil composition contains no more than about 0.03 weight percent of phosphorus, based on the total weight of the natural gas engine lubricating oil composition, and further wherein the natural gas engine lubricating oil composition is substantially free of any alkali metal-containing detergents.

2. The method of claim 1, wherein the natural gas engine lubricating oil composition further comprises sulfurized isobutylene.

3. The method of claim 1, wherein the natural gas engine lubricating oil composition prevents or inhibits exhaust valve seat recession in the natural gas fueled engine greater than or comparable to a corresponding natural gas engine lubricating oil composition in which the one or more alkaline earth metal salts of an alkyl-substituted hydroxybenzoic acid is replaced with an alkaline earth metal-containing phenate detergent.

4. The method of claim 1, wherein the natural gas engine lubricating oil composition has a sulfated ash content of about 0.15 to about 0.3 wt. % as determined by ASTM D 874.

5. The method of claim 1, wherein the natural gas engine lubricating oil composition is substantially free of any molybdenum-containing compounds.

6. The method of claim 1, wherein the natural gas engine lubricating oil composition contains from about 0.005 to about 0.03 wt. % of phosphorus, based on the total weight of the natural gas engine lubricating oil composition.

7. The method of claim 1, wherein the natural gas engine lubricating oil composition has a sulfated ash content of about 0.12 to about 1.0 wt. % determined by ASTM D 874.

\* \* \* \* \*